

F. I. DU PONT.

METHOD OF SOLIDIFYING CRYSTALLIZABLE MIXTURES WITHOUT SUBSTANTIAL CRYSTALLIZATION.  
APPLICATION FILED JAN. 31, 1910.

1,007,276.

Patented Oct. 31, 1911.

2 SHEETS-SHEET 1.



WITNESSES:

*Daniel Webster, Jr.*  
*A. M. Ryan.*

BY

INVENTOR  
*Francis T. Duson*  
ATTORNEYS  
*Henry C. Tracy*

F. I. DU PONT.

METHOD OF SOLIDIFYING CRYSTALLIZABLE MIXTURES WITHOUT SUBSTANTIAL CRYSTALLIZATION.  
APPLICATION FILED JAN. 31, 1910.

1,007,276.

Patented Oct. 31, 1911.

2 SHEETS—SHEET 2.

FIG. 2.



# UNITED STATES PATENT OFFICE.

FRANCIS I. DU PONT, OF WILMINGTON, DELAWARE, ASSIGNOR TO E. I. DU PONT DE NEMOURS POWDER COMPANY, OF WILMINGTON, DELAWARE, A CORPORATION OF NEW JERSEY.

## METHOD OF SOLIDIFYING CRYSTALLIZABLE MIXTURES WITHOUT SUBSTANTIAL CRYSTALLIZATION.

1,007,276.

Specification of Letters Patent. Patented Oct. 31, 1911.

Original application filed September 24, 1909, Serial No. 519,318. Divided and this application filed January 31, 1910. Serial No. 540,951.

To all whom it may concern:

Be it known that I, FRANCIS I. DU PONT, a citizen of the United States, residing at Wilmington, county of New Castle, and State 5 of Delaware, have invented a new and useful Improvement in Methods of Solidifying Crystallizable Mixtures Without Substantial Crystallization, of which the following is a full, clear, and exact description, reference 10 being had to the accompanying drawings, which form a part of this specification.

In the manufacture of "black powder" from an initial mixture of the ingredients when in a dissolved, liquid, or semi-liquid 15 condition produced by solvents or heat or both, it is necessary to return the material to a solid condition without substantial crystallization. It is also necessary in the process to which this application refers to 20 do this in such a way that in the return of the ingredients from the liquid condition, masses can be formed of any desired size or shape and of sufficient hardness to form what are known as grains of powder. Some 25 of the ingredients of this powder are rendered soluble by a liquid, other ingredients by heat. I first subject the dissolved, liquid or semi-liquid mixture, to the action of heat and rubbing or abrasion. An apparatus by 30 which this step may be carried out is described and illustrated in Letters Patent No. 944,500, issued to me December 28th, 1909. This action will have no effect upon such ingredients as are brought to a liquid condition 35 by heat, and were it attempted to bring to a solid condition by this operation all of the ingredients which are not brought to a liquid condition by heat, the material delivered would either be in the form of dust 40 or of lumps of insufficient hardness, or more probably a mixture of such lumps and dust, which product would be altogether inferior, if not useless, for the purpose for which ordinary blasting powder is used.

The object of my invention is to bring the material, which is delivered in a liquid or semi-liquid condition by the apparatus described in my aforesaid patent, to a plastic condition and to do this without substantial 45 crystallization of the materials which are brought into the liquid state by solution, or of those materials which are

brought into the liquid state by heat. The mass after admixture in a fluid or semi-fluid condition is subjected to heat while working such mass during said treatment. The effect of this is to bring into a partially solid condition those ingredients which are rendered liquid by a solvent, the results being accomplished by the evaporation of the solvent 55 during a rapid agitation of the mass. This treatment, however, does not have this effect upon the ingredients rendered liquid by heat. For instance, take black powder, an example of the ingredients is 73 parts nitrate of soda, 65 16 parts charcoal and 11 parts sulfur, in such composition the liquid sulfur will not be solidified or partially solidified by this treatment. Also it is not desirable to carry this treatment far enough to solidify the 70 nitrate of soda, because for the reason above given.

The treatment of heat and working just described may be carried on in an apparatus and in the manner described, illustrated and claimed in the patent before mentioned.

The present invention relates to a process for completing the partial solidification, that is, that stage of the solidification which is 80 required for the formation of grains, these grains being cut or molded from a plastic mass having so small a per cent. of moisture that further evaporation of this moisture will not produce crystallization.

I have discovered that if I take the mixture after it has passed through the evaporator and form it into a thin sheet, which sheet must be for the best results as thin as it can be formed, and when in such thin 90 sheet, subjected to cooling action the material is rapidly cooled and solidified, and all the material practically simultaneously so chilled and solidified, and the solidification of the ingredients of the previous treatment 95 completed, and the solidification of the other ingredients obtained, all without crystallization. The material thus solidified may then be broken up, and if grains are desired to be produced, formed into a sheet of the desired 100 thickness and the grains cut therefrom.

I will now describe an apparatus for carrying out my method or process, and which apparatus forms the subject matter of an

application filed by me September 24th, 1909, Serial No. 519,318, of which this application is a division.

In the drawings: Figure 1 is a general view of my invention, with some of the parts in elevation and others in section. Fig. 2 is a section on the line 2—2, Fig. 1. Fig. 3 is a detailed view of a portion of the apparatus adjacent to the point of reception of the material upon the roller. Fig. 4 is an enlarged section of the mechanism for removing the powder from the carrying roller and forming it into the ultimate sheet or strip.

5 *a, a*, are the evaporating tubes of the evaporator, as described in my application before mentioned, and also described in an application filed by me July 28, 1909, Serial No. 510,070. The material passes from 10 these evaporators into a stack *b*, having the chamber *c*. The carrying roller *d*, which is revolved by appropriate mechanism in the direction indicated by the arrow, forms the bottom of this chamber *c*. The forward wall 15 of chamber *c* is cut away to admit the pressing roller *e*, which is revolved in the direction of the arrow. The peripheral speed of the rollers *d* and *e* is the same. The tendency of this roller *e* is to press the material 20 in the chamber *c* onto the face of the roller *d*. On the other hand, the material is of such character that its tendency is to follow the roller *e* as well as the roller *d*. In order to obviate this last mentioned condition 25 I use what I term a spreader and scraper *f*. This scraper and spreader *f* is pivoted and backed up by the spring *g*. This combined scraper and spreader *f* has a portion contacting with the surface of the 30 roller *e* to prevent the material following the roller *e*. As shown, this has a knife edge. It is also provided with a projecting lip *f'* which is spaced a distance from the surface of the roller *d* equal to the distance 35 between the surfaces of rollers *d* and *e* at their nearest point. By this arrangement the material is, by the action of the roller *e*, spread upon the roller *d*, and the thickness of the sheet determined by the distance 40 between the rollers *d* and *e*. Further, the scraper and spreader prevent the material following the roller *e* and also maintain the thickness of the sheet the same as that of the distance between the rollers. As stated, 45 the roller *d* is a skeleton roller, having the internal chamber 5.

50 *h* is a pipe leading from a source of water supply or cooling fluid, not shown. The pipe *h* passes through the hollow hub of the roller *d* and connects with the pipe *i*, which passes up vertically in the chamber 5, and terminates in the branch *j*, having the nozzles or sprayers *k*.

55 *l* is a pipe leading from the lower portion of the chamber 5, connecting with the pipe

*m*. The pipe *m* also passes through the hub of roller *d* and is connected with a suction pump. When water passes from the pipe *h*, under pressure, it is forced out through nozzles *k* and sprayed against the inner surface of the roller *d*, thus chilling the surface of the roller *d* and chilling the powder strip as it passes around with the wheel. The roller *d* is driven by the worm 1 and worm wheel 2. The water will flow by gravity to the bottom of the chamber 5, and is withdrawn by the pump, acting through pipes *m* and *l*.

70 As stated before, the sheet from the roller *d* is too thin to be used in the subsequent steps in the manufacture of the powder into grains. I therefore have provided, as is necessary in this apparatus, mechanism for the purpose of forming this thin sheet into a sheet of proper thickness to be cut into 75 powder grains.

80 Near the lower surface of the roller *d* I provide the rollers *o*, *p*, and *q*. The roller *o* revolves in the same surface direction and at the same surface speed as the roller *d*. The roller *q* revolves in the opposite direction and at a surface speed to be determined by the desired thickness of the ultimate powder strip, as will hereinafter be more 85 fully described. As these two rollers *q* and *o* revolve in opposite directions the powder sheet upon the roller *d* will, when it reaches those rollers, be, by their reverse action, crowded between them into the space as shown. The scraper *t*, backed up by the 90 spring *u*, prevents any powder passing beyond the roller *q*. Between the rollers *o* and *q* is the roller *p* revolving in a direction opposite to the roller *q*. The material crowded between the rollers *o* and *q* is prevented 95 from passing out between the rollers *o* and *p* by means of the scraper and cleaner *v*, backed up by the spring *w*. As the drawings show, the scraper and cleaner *v* contacts with the roller *o*, as that is the roller 100 which will tend to carry the material around in the direction between the rollers *o* and *p*. In like manner, the scraper and cleaner *t* contacts with the surface of the roller *d*, as that roller is the one which will tend to 105 carry off and prevent the material being brought into the space between the rollers *q* and *o*. The rollers *p* and *q* are separated from each other at a distance equal to the thickness of the desired powder strip and 110 their peripheral velocities are determined upon the basis of the thickness of the powder strip desired and the quantity acted on.

115 Contacting with the roller *q* is a scraper and spreader *z*, quite similar to the scraper and spreader *f*, before described. It, like the scraper *f*, has the scraping surface or edge, which contacts with the roller *q*, and the projecting lip *z'* which is spaced from the roller *p* a distance equal to the distance 120

between the rollers *p* and *q* at the nearest points said rollers approach each other. By this construction the powder mass in the space between the rollers *o* and *q* will pass out between the rollers *p* and *q* and will be prevented from following the roller *q* by the scraping surface of the scraper and spreader *z*, and be maintained by the lip *z'* at the proper thickness. The action is thus a formative one between the rollers *p* and *q*, these forming a spreading and holding action between the lip *z'* and the roller *p*.

Finally, the powder strip is released from the roller *p* by means of the scraper *x*, the scraping surface of which contacts with the roller *p* beyond the point of action of the lip *z'*. This scraper *x* is also provided with a projecting lip *x'* to carry the powder fully clear of the scraper itself so that it will move or pass free from said scraper. The scraper *x* is held in operative position by the spring *y*.

Having now fully described my invention, what I claim and desire to protect by Letters Patent is:

1. The hereinbefore described method of solidifying crystallizable mixtures rendered liquid or semi-liquid by solvents and heat, without substantial crystallization, which consists in subjecting the mixture to the action of heat and rubbing to remove the solvents, then forming said material into a thin sheet, then chilling said sheet.

2. The hereinbefore described method of solidifying crystallizable mixtures rendered liquid or semi liquid by solvents and heat, without substantial crystallization, which consists in subjecting the mixture to the action of heat and rubbing to remove the solvents, then forming said material into a thin sheet, then chilling said sheet and then breaking up said sheet and by pressure forming the material into a sheet of the desired thickness.

3. In the method of solidifying crystallizable mixtures of the character described without substantial crystallization, forming the mixture into a thin sheet, then chilling said sheet, then breaking up said sheet, and then forming the material into a sheet of the desired thickness.

4. In the method of solidifying crystallizable mixtures of the character described without substantial crystallization, forming the mixture into a thin sheet, chilling said sheet, then forming material into a sheet of greater thickness than the first mentioned sheet.

In testimony of which invention, I have hereunto set my hand, at Philadelphia, on this 28th day of January, 1910.

FRANCIS I. DU PONT.

Witnesses:

M. M. HAMILTON,  
A. M. URIAN.